

April 5, 1932.

C. S. HAMM

1,852,158

## PAPER MANUFACTURE

Filed April 10, 1930.

2 Sheets-Sheet 1



Inventor

Charles S. Hamm

१३४

Marcel and Noe

Attorney S

April 5, 1932.

C. S. HAMM

1,852,158

## PAPER MANUFACTURE

Filed April 10, 1930

2 Sheets-Sheet 2



Inventor

Charles S. Hamm

Maréchal and Rose  
Attorneys

## UNITED STATES PATENT OFFICE

CHARLES S. HAMM, OF DAYTON, OHIO, ASSIGNOR TO MEAD PAPERBOARD CORPORATION, OF WILMINGTON, DELAWARE, A CORPORATION OF DELAWARE

## PAPER MANUFACTURE

Application filed April 10, 1930. Serial No. 443,213.

This invention relates to the manufacture of paper, and the like, and particularly to the preparation of pulp for use in such manufacture.

One of the principal objects of this invention is to provide a method of treating fibrous materials, such as deciduous wood, to form a superior pulp having high strength with a large yield, and in which desired uniformity of the pulp product is obtained, while insuring ease of handling of the material and the formation of paper therefrom at desired high speeds.

Another object of this invention is to provide a method of cooking fibrous materials of this character, in which desired control of the cooking treatment is effected by proportioning of the chemicals used in the cook to give a product of desired quality and uniformity.

Another object of the invention is to provide a method of extracting tannic acid from deciduous wood, such as chestnut chips, and then pulping the extracted or leached wood, in which the leaching treatment is coordinated with the subsequent pulping treatment to give an extract of desired purity and a pulp product of controlled quality.

Still another object of this invention is to provide apparatus for carrying out the above method, which apparatus is simple in construction, and highly effective and readily controlled in operation.

Other objects and advantages of the invention will be apparent from the following description, the accompanying drawings and the appended claims.

In the drawings, in which like characters of reference designate like parts throughout the several views thereof—

Fig. 1 is a diagrammatic side elevational view of a portion of the apparatus for carrying out the method of this invention;

Fig. 2 is a diagrammatic side elevational view of the remaining portion of the apparatus, Fig. 1 showing that portion of the apparatus to the left of the line A—A and Fig. 2 that part to the right of such line; and

Fig. 3 is a diagrammatic side elevational view at right angles to Fig. 1 of a portion of the apparatus.

Referring to the drawings, in which a preferred embodiment of apparatus for carrying out the method of this invention is disclosed, a chipper for reducing pieces of wood or logs to chips is indicated at 10. This chipper may be of conventional construction, and is provided with a feeding inlet 11 through which the logs are introduced and a discharge outlet 12 through which the chips subdivided to a suitable size are discharged onto a traveling conveyor 13. The conveyor 13 may be of any suitable type, such as that having a trough 14, on the surface of which travels an endless chain 15 supported by rolls 16 and 17 and carrying transverse drags 18, which serve to drag the chips up the trough in the direction of the arrow and discharge them onto a second traveling conveyor 20.

The conveyor 20 is constructed similarly to the conveyor 13 in that it is provided with a trough 21 within which travels the endless chain or belt 22 supported by rolls 23 and 24 and carrying transverse drags 25. The trough 21 is provided with spaced openings 26 adapted to be controlled by suitable slide valves 27, through which the material moved along the trough 21 may fall into inclined chutes 28. Each of the chutes 28 is inclined downwardly and also laterally so as to clear the path of return of the endless conveyor 20 belt. The lower ends of the chutes 28 discharge as indicated at 29 into a plurality of leaching tanks 30, in which the leaching of the chips for the extraction of tannic acid is accomplished. The arrangement shown is known as an "open tank" leach, in which the leaching tubs are open to atmosphere and the leach is carried out at atmospheric pressure; but closed tanks or autoclaves may be used, if desired, and the leaching carried out under pressure greater than atmospheric. While three leaching tanks 30 are illustrated in the drawings, it is to be understood that this is merely for convenience in illustration and that a larger number of such leaching tanks is generally used. The leaching tanks are arranged in line, so that the common conveyor 20 may supply chips to all of them.

Each leaching tank comprises a cylindrical tub having a bottom 31 and a spaced perfo-

rate false bottom 32, which may be constructed of lattice work. Chips are fed into the tank 30 until it is filled to the desired level. The leaching operation is then begun by the introduction of sprays of water onto the chips from valve controlled pipe lines 33, and the leaching liquid and chips are heated by the introduction of steam at valve controlled steam pipes 34. Preferably, when a number of leaching vessels are used in series, the leaching liquid is passed through the vessels in a counter-current flow. That is, the most concentrated leaching liquor, or water solution of extracted tannic acid, is passed into contact with the chips in a leaching tank which has just been connected in the series, so that the concentrated liquor will be brought into contact with fresh chips; while the tank which has been connected in the series for the longest time is treated with fresh water so that an effective extraction is obtained.

The leaching tubs may thus be operated in sequence or in alternation; as one leaching tub which has been in leaching operation for the longest time is cut out, a new leaching tub with fresh chips is brought into operation, permitting the leached chips in the tub which has been cut out to be removed. This tub is then refilled with fresh chips, and is ready to be again cut in at the other end of the leach liquor line, that is at the fresh water end. The water introduced into the first tub of the series, as by the pipe 33, percolates through the chips within the leaching tub and discharges through valve controlled pipe 35. Each valve controlled pipe 35 communicates with suitable conventional piping (not shown) by which the liquor discharging from a first tub may be passed to the second tub of the series, and so on through the group of leaching tanks which are connected in series. For example, ten tanks may be run in series with counter-flow circulation. The concentrated leach liquor from the last tub of the series is discharged into a leach liquor outlet pipe 36, which communicates with all the tubs and leads to a storage tank (not shown), from which the leach liquor may be supplied to the evaporators and concentrated to produce the tannic extract of commerce.

When a leaching tub is cut out of the leaching operation, the extracted chips therein are then permitted to drain for a time through the perforate grid or lattice work 32, the drained liquor being removed through pipes 35 and 36, and then the drained chips are removed at a controlled rate from the tub. As shown, each leaching tub is provided with a "leach caster", which comprises a central vertical shaft 40 supported in suitable bearings and driven through gears 41 and 42 from a shaft 43, which is adapted to be connected to a suitable source of power by a clutch (not shown), so that the shaft

43 and leach caster may be brought into operation as desired in each particular tank. A stirring arm 44 is slidably mounted on the shaft 40 for vertical movement thereon and is keyed thereto so as to rotate with shaft 40. The stirring arm 44 carries a plurality of depending inclined blades or fingers 45 which are so inclined as to move the chips toward the periphery of the tank upon rotation of the shaft 40 and arm 44. The construction is such that the arm 44 rests on the surface of the chips within the leaching tub and slides vertically down the shaft 40 as the level of the chips falls due to discharge of the chips from the tub, the arm thus rotating with the shaft 40 while resting on the surface of the chips.

Adjacent the periphery of each tank 30, a port or opening 47 is provided in the perforate grid 32, which is adapted to be opened or closed by a sliding plate valve 48. The opening 47 is in alignment with a discharge pipe 49 extending from the bottom of the tank, and adapted to discharge onto a traveling conveyor 50. Each discharge pipe 49 is also controlled by a sliding plate valve 51. When the draining operation in the leaching tank is completed, the valve 35 is closed and the valves 48 and 51 opened. The leach caster is then started, serving to move the chips to the periphery of the tank and out through the discharge pipe 49. The rate at which the chips are fed to the periphery of the tank and discharged is controlled by the rate of rotation of the shaft 40, which may be controlled from the line shaft in any suitable manner, such as by a variable cone pulley drive from a line shaft to the shaft 43.

Conveyor 50 is constructed similarly to conveyor 20 and is arranged transversely beneath the line of leaching tanks so as to receive the extracted chips discharged from each of the tanks. Generally only one or several of the leaching tanks will be discharging at any particular time, the remaining tanks being in leaching or draining operation at such time. Consequently a controlled rate of feed of the drained chips is provided from the leach tanks, and these chips are carried in the direction of the arrow by conveyor 50 supported on suitable rolls 52 and 53. This conveyor discharges onto another conveyor 54, which is supported on an inclination to the horizontal by rolls 55 and 56 and serves to elevate the chips and discharge them into the interior of a rotary cylindrical screen indicated diagrammatically at 58. Screen 58 is inclined from the feeding end 59 to the discharge end 60 thereof, so that the material feeds through the screen as it is rotated and discharges therefrom onto another conveyor 61. A container 62, built up beneath the screen 58 to receive the fine material or screenings passing there-

through, has a lower hopper portion 63 feeding into another conveyor 64.

It is found that a better grade of pulp is produced when the leached chips are screened to remove the finer sawdust and impurities prior to the pulping operation. The screenings are quite satisfactory for boiler fuel, so that the conveyor 64 may be arranged to convey them in the direction of the arrow to the boiler fuel supply, or other point of discharge.

Conveyor 61 moves the screened material in the direction of the arrow to supply the cooking tanks or digesters. As shown, a plurality of spherical digesters 65 are mounted in line, each for rotation about horizontal trunnions or bearings 66. Positioned above each digester in a storage bin 67 terminating in a converging lower end or hopper 68 controlled by slide valve 69. Each digester is provided with a cover plate 70 removably bolted thereto, and so positioned as to be adapted to be brought into alignment with the valve controlled opening of the feeding hopper 68. Trough 71 of conveyor 61 has a plurality of spaced openings 72 controlled by sliding plates 73, through which the chips moved along trough 71 may fall into chutes 74 discharging into the respective feeding hoppers 67. The chutes are downwardly and laterally inclined so as to be removed from the path of travel of the lower returning portion of the endless conveyor. The storage bins 67 are adapted to be maintained filled, or with a sufficient supply of chips, so as to provide a complete charge for a digester. In filling, each digester 65 is rotated about the trunnion 66 until the cover plate 70 is brought into alignment with the discharge hopper of the storage bin 67. The cover plate 70 is then removed, and the valve 69 opened to allow the chips to feed into the digester until a full charge is supplied thereto. The cover plate 70 is then replaced and the cooking commenced.

The leached chips are cooked with an incomplete digestion or "semichemical" cook which gives a high yield and a product of good strength. In the semichemical cook, very satisfactory results are secured with a cooking liquor containing a normal sulphite and an alkali metal salt of a weakly ionized polybasic acid, such as a mixture of sodium sulphite and sodium carbonate. The cook is generally carried out in two stages, although it may be carried out in a single stage. The cooking liquor is introduced from suitable liquor supply tanks (not shown) through piping passing through the hollow trunnions 66 to submerge the chips, and the temperature is brought up to approximately 125° C. to 150° C. with steam for a length of time to secure desired impregnation of the liquor within the wood. A treating time of about two hours gives satisfactory results in

this first stage. The unabsorbed liquor is then drawn off or blown back into the liquor tanks, and the liquor saturated material remaining in the digester is raised to a higher temperature of 160° C. to 180° C. for a period of time, generally about three to four hours. At the completion of the cook, the softened chips are discharged into a dump tank 75 positioned therebeneath.

It has been found after prolonged commercial operations that the pulping operations are affected by the leaching treatment given in the step of extracting tannic acid from the chips, so that for best results the leaching treatment and the subsequent pulping treatment are coordinated with each other. In accordance with the present invention, the chips are subjected to a controlled leach so as to give a uniform residue, or leached chips of uniform composition, as a result of the leaching operation. The degree of leaching treatment is dependent upon the time, temperature, pressure and volume of leaching liquid or water used per unit weight of chips. By increasing the time of treatment, the leaching effect is increased; that is, a greater proportion of the tannic acid and other readily soluble constituents of the wood are dissolved out of the chips. Similarly by increasing the temperature or pressure used in the leaching operation, or by using a greater volume of leaching liquor per unit weight of chips, the leaching effect is correspondingly increased. These conditions of leaching, namely, time, temperature, pressure and volume of leaching liquor, are therefore controlled so as to give a resulting leached chip which has a substantially uniform composition or residue, this being termed herein for purposes of description a "residue controlled" leaching operation.

It is also found that the character of the pulped material produced by the digestion of the leached chips, as well as the character of the ultimate sheet formed from such pulp is also dependent upon the cooking or digesting operation. The degree of cooking treatment is dependent upon the quantity and proportioning of the chemicals used, and the time, temperature and pressure of the cooking operation. The cook is coordinated with the leaching treatment by suitably controlling and interconnecting these cooking conditions in accordance with the character of the residue resulting from the leach. This control and coordination of the quantity and proportioning of the chemicals, the time, temperature and pressure of the cook with respect to the inherent characteristic effect of each, and also with respect to the pulping characteristics of the residue controlled chips, is termed herein for purposes of description a "reaction controlled" chemical cook.

In addition, various woods require different cooking operations to give substantially

the same reactivity to the subsequent chemical treatment. By controlling the leaching effect so as to give a uniform leached product or residue, a subsequent uniform cooking or pulping treatment may be given for a particular material, thereby assisting materially in the carrying out of this method in actual practice. By maintaining the leaching operation substantially constant and the cook correspondingly so, then predetermined characteristics in the cooked chips may be secured, so that the subsequent steps in the completion of the pulping operations and in the satisfactory utilization of the pulp to form the desired sheet may be intelligently and readily controlled in commercial operations.

Where chestnut wood is used, and the leached chestnut chips resulting therefrom, are then utilized in the manufacture of paper pulp, it is found preferable that the extent of leaching be not increased materially over seventy hours. On the other hand, it is desirable to give a sufficiently long immersion of the chips during the leaching operation to obtain increased extraction, or a greater yield of tannic acid, without lowering the purity of the extract. Satisfactory results have been secured in actual commercial operations in several plants using an open tank leach with a leaching time varying from about thirty to seventy hours, the leaching temperature varying from between 140° F. to 212° F. and using approximately 1500 to 1800 gallons of water per long cord of chestnut chips.

It is also found that the proper quantities or relative amounts of the normal sulfite and the carbonate or other alkali metal salt of a weakly ionized polybasic acid such as sodium bicarbonate, sodium borate, and the like, should be utilized in the subsequent semi-chemical cooking operation. The final characteristics of the ultimate product are not only affected, but also the handling of the material in the subsequent formation on the paper machine, if the proper relative amounts are not maintained, as well as the proper coordination of this cooking step with the previous leaching operation.

Sufficient sodium carbonate, or other alkali metal salt of a weakly ionized polybasic acid, should be used to neutralize the organic or pyrolygneous acids present in the leached chips and given off during the cook, and to maintain a slight alkalinity of the cooking liquor. The efficacy of the cooking liquor, or the sodium sulfite as a cooking agent, appears to be enhanced by the maintenance of substantial neutrality of the cooking liquor during the cook, a slight alkalinity being preferred to any acidity. It has been found that the sodium sulfite is the active cooking agent and gives under such conditions the desired pulp products, and that the function of

the sodium carbonate is to maintain the desired neutrality or slight alkalinity of the cooking liquor. The sodium carbonate should therefore be used in a controlled proportion to give this most effective condition of neutrality or slight alkalinity, but it should not be used in sufficient proportion to materially affect or reduce the cooking efficacy of the sodium sulfite. Moreover, it is found that where the carbonate is present in quantities materially in excess of that required for neutralization of the acids, then a pulp product of inferior quality is produced. At the same time, a controlled amount of sodium sulfite, or other alkali metal sulfite such as potassium sulfite, should be used in connection with the controlled amount of sodium carbonate in order to give a cooked product of the desired characteristics. With wood of this character, a certain proportion of the acid content, such as tannic acid, is left in the chip residue resulting from the leaching operation; and other acid may be formed by reaction during the cook. By providing a controlled leaching operation so as to give a uniform residue, the proportions of chemicals used in the cook can thus be maintained uniform and in proper amounts to secure this desired neutralizing and cooking action for a given chip residue.

If it is desired to increase the cooking effect, this may be accomplished by increasing the proportion of sodium sulfite used, while maintaining the sodium carbonate constant at that amount which effects the neutralization of the liberated acids and the maintenance of a slight alkalinity of the cooking liquor. If it is desired to decrease the cooking effect, this may be brought about by decreasing the proportion of sodium sulfite, the carbonate being maintained constant. By increasing the quantity of carbonate for a given chip residue, while maintaining the quantity of sulfite constant, it is found that the net cooking effect is decreased. It is more efficient to vary the proportion of sodium sulfite used within the above range to vary the cooking effect, as this leaves the carbonate at the proper amount for neutralization of the acids of a particular chip residue. By increasing the quantity of carbonate materially above this amount, the cooking efficacy of the sulfite is reduced and a poorer pulp product produced, this obviously being an inefficient way of decreasing the cooking effect.

Where the quantities of chemicals used are altered, such as for digesters of different sizes and consequently for different weights of chestnut chips leached in the manner described above, the carbonate should be increased or decreased in accordance with the acid content of the chips to maintain the desired neutrality of the cooking liquor, while the sulfite should be increased or decreased in proportion to the quantity of the wood.

and the character of the pulp product desired, and these chemicals should not be arbitrarily increased or decreased like amounts, if the cooking conditions are to be maintained approximately the same. By the maintenance of coordinated conditions in the residue controlled leaching operation and the reaction controlled cooking operation, and by the maintenance of the proper relative quantities of chemicals in the cooking operation, a pulp can be uniformly produced in commercial operation which has high strength, good yield, and which is susceptible of formation on a forming machine at high speeds. Where this pulp is used in the manufacture of so-called corrugated board, it has been found in actual operation that the pulp can be passed over a forming machine including a conventional corrugating machine at a speed of 250 feet per minute or more without operating difficulties.

As an example of an operation giving very satisfactory results, a leaching time in an open tank leach of about thirty-four to forty-two hours at a temperature of about 160° F. to 212° F. using about 1800 gallons of water per long cord of chestnut chips, is mentioned. This gives an extract of desirably high purity, for example a purity of at least 70 as measured on the arbitrary scale used in the extract industry. The leached chip residue resulting from this leaching operation is then cooked in the manner described above with a cooking liquor containing about 2000 to 2100 pounds of sodium sulfite (calculated as sodium carbonate) and about 650 to 700 pounds of sodium carbonate for about 8½ short cords of the leached chestnut chips. The chemicals may of course be used in different relative amounts within a certain operating range and in accordance with the pulp product desired. Thus in actual commercial operations, with a certain character of chestnut chip treated, and with the leaching operations as specified above, satisfactory results have been obtained where these chemicals are present in the cooking liquor in the proportion of substantially 2.5 to 3.7 parts by weight of sodium sulfite to one part by weight of sodium carbonate (both chemicals being calculated as sodium carbonate). Thus with a digester having a capacity of about 8½ short cords of leached chestnut chips (weighing on a dry basis about 19,000 to 20,000 pounds) satisfactory results in commercial operation have been secured where substantially 1750 to 2350 pounds of sodium sulfite (calculated as sodium carbonate) and substantially 650 to 700 pounds of sodium carbonate have been used, with cooking conditions of time, temperature and pressure as set forth above.

In actual commercial operations, by using a definite substantially constant leaching operation for the different types of chestnut wood encountered, it is found that a relatively

constant tannic acid content remains in the chip residue for the different types of wood, actual tests showing a tannic acid residue varying from about 1¼ to 1¾%. As a matter of convenience in such commercial operations, a slight excess of carbonate, say about fifty pounds per digester, is used in the cooking liquor over that required for neutralization of the minimum acid content of the chip residue. This excess is sufficient to take care of the normal variation of about ½% in the tannic acid content encountered, and to maintain the desired neutrality or slight alkalinity of the cooking liquor; at the same time, this slight excess is not sufficient to materially affect the cooking efficacy of the relatively large amount of sulfite or the character of the pulp product obtained.

Altering the leaching operation has the effect of removing variable quantities of materials in the leaching step, which throws disturbances in the reaction stage. For a certain set of conditions in the leaching stage, a uniform residue may be secured with a particular wood, and this residue may then be tested to ascertain its retained acid and non-cellulose content. The subsequent cooking may then be properly coordinated therewith, inasmuch as when the residue content of the chip is known, a proper cooking operation for that residue content will give a pulp of the desired and uniform quality, and the conditions of cooking for a particular residue content may be readily ascertained by experiment or experience. Consequently, it is only necessary in the commercial operations to choose the properly coordinated cooking operation for a certain ascertained residue content, so as to obtain the desired ultimate product. And by controlling the leaching operation so as to maintain this residue content uniform at an ascertained value, the entire operation may be carried out in practice with relatively unskilled labor and without extended chemical analysis for each particular operation, and a uniform tannic acid extract of desired purity and a uniform pulp product of controlled quality obtained.

As an example of altered conditions, a leaching time of about sixty to seventy hours at a temperature of about 160° F. to 212° F. and using about 1800 gallons of water per long cord of chestnut chips, gives satisfactory results with the employment of a subsequent cook in a liquor containing about 1800 to 1900 pounds of sodium sulfite (calculated as sodium carbonate) and about 625 to 675 pounds of sodium carbonate per 8½ short cords of leached chestnut chips. The figures given above refer to open tank leaches. Where autoclave leaches are used, satisfactory results have been obtained with a temperature range of about 160° F. to 250° F., using about 1000 to 1200 gallons of water per long cord of chestnut chips.

The dump tanks 75 are arranged in line beneath the spherical digesters 65, each to receive material dumped from its respective digester. The material at the completion of the cook is softened but still maintains to a large degree its chip form. Where the ultimate product is board, such as corrugated board, the digester is preferably not blown, but is merely dumped so that the softened material is not shredded or pulped at this stage but is maintained in chip form, whereby it is easily handled at high density, i. e. low moisture content. The mass of softened chips discharged into each dump tank 75 is then washed to remove residual liquor. This may be accomplished by the introduction of sprays of washing liquid through valve controlled pipes 76, the liquor draining through a perforated partition or latticework 77 within the bottom of the dump tank, and escaping by a valve controlled outlet pipe 78 communicating with a drain 79.

Each dump tank 75 is provided with means for feeding the softened and drained chips at a controlled rate to subsequent treating apparatus, such as a rod mill or other mechanical disintegrating apparatus for reducing the softened chips to pulp. As illustrated, each dump tank 75 is provided with a leach caster construction including a central vertical shaft 80 carrying a sliding arm 81, the shaft 80 being driven by intermeshing gears 82 and 83 from a driven shaft 84 adapted to be connected to a suitable source of power. A valve controlled opening 86 is provided in the grid 77 in alignment with a valve controlled discharge pipe 87, so that drained chips may be discharged at a controlled rate therethrough onto a traveling conveyor 88 common to all the dump tanks and which carries them in the direction of the arrow to the subsequent treating apparatus. The digesters are preferably cooked in rotation, so that one or several are cooking while another is being dumped. Thus the softened chips in one dump tank, after washing and draining, may be fed slowly and at a controlled rate from the dump tank by the leach caster during the time that another batch of chips is being cooked in its respective digester, and still another batch of chips in another dump tank is being washed and drained.

While the method herein described, and the form of apparatus for carrying this method into effect, constitute preferred embodiments of the invention, it is to be understood that the invention is not limited to this precise method and form of apparatus, and that changes may be made in either without departing from the scope of the invention which is defined in the appended claims.

What is claimed is:

1. In the pulping of acid containing deciduous woods, the method which comprises leaching the woods to extract a substantial

proportion of the soluble contents therefrom while leaving a proportion of the more difficultly soluble acid content in the woods to maintain the purity of the extract, cooking the previously leached woods in a liquor containing a normal sulfite and an alkaline material, the normal sulfite being controlled as to amount to give a controlled cooking action such as to soften the woods without pulping so as to provide for subsequent disintegration to pulp, and the quantity of alkaline material being controlled in accordance with the residual acid content of the woods to neutralize the residual acid in the leached woods and such acid as may be generated during the cooking action and insufficient to materially affect the cooking action of the normal sulfite or deleteriously affect the pulp product.

2. In the pulping of chestnut chips, the method which comprises leaching the chips to extract a substantial proportion of the soluble contents therefrom while leaving a proportion of the more difficultly soluble acid content in the chips to maintain the purity of the extract, cooking the previously leached chips with a cooking liquor containing an alkali metal sulfite and an alkali metal carbonate in the proportions of substantially 2.5 to 3.7 parts by weight of the alkali metal sulfite (calculated as sodium carbonate) to one part by weight of the alkali metal carbonate (calculated as sodium carbonate), and increasing or decreasing the quantity of the alkali metal sulfite within the proportions specified while maintaining the quantity of the alkali metal carbonate substantially constant to respectively increase or decrease the cooking effect.

3. In the extraction of tannic acid from acid containing deciduous wood chips and the pulping of extracted wood chips, the method which comprises leaching the deciduous wood chips with water to extract a substantial proportion of the soluble contents therefrom while leaving a uniformly controlled acid residue in the chips so as to maintain the purity of the extract, then subjecting the leached chips to a controlled pulping treatment including cooking in a liquor containing a normal alkali metal sulfite and the alkali metal salt of a weakly ionized polybasic acid, the pulping treatment being coordinated with the previous leaching treatment by varying the quantity of the alkali metal salt of a weakly ionized polybasic acid used in the cooking liquor in accordance with the acid residue of the leached deciduous wood chips to maintain substantial neutrality or a slight alkalinity of the cooking liquor during the cooking operation, and varying the quantity of normal alkali metal sulfite used in accordance with the quantity of wood and the pulp product desired.

4. In the extraction of tannic acid from chestnut chips and the pulping of extracted

5 chips, the method which comprises leaching the acid containing chestnut chips in water at substantially atmospheric pressure for a period of time not exceeding 70 hours to extract a substantial proportion of the soluble 10 contents therefrom while leaving a proportion of the more difficultly soluble acid content in the chips to maintain the purity of the extract, and then subjecting the leached chips 15 to a pulping treatment including cooking with a cooking liquor containing substantially 2.5 to 3.7 parts by weight of sodium sulfite (calculated as sodium carbonate) and one part by weight of sodium carbonate, the 20 cooking treatment being controlled to coordinate the same with the previous leaching treatment by controlling the quantity of sodium carbonate within the proportions specified in accordance with the residual acid 25 content of the leached chips, and by controlling the quantity of sodium sulfite within the proportions specified in accordance with the quantity of wood and the degree of softening desired in the cooking operation.

30 5. Apparatus of the character described, comprising in combination, a leaching tank for extracting tannic acid from wood chips, draining means for said leaching tank, means for discharging leached chips at a controlled 35 rate from said tank, a storage bin, conveying means for transporting said chips as discharged from said leaching tank to said storage bin, a digester, and means for introducing the chips from said storage bin into said digester.

35 6. Apparatus of the character described, comprising in combination, a plurality of leaching tanks arranged in line, a conveyor extending transversely of said tanks for receiving material discharged from each of said 40 plurality of leaching tanks, a plurality of digesters, storage bins for said digesters positioned in line and in feeding relation with said digesters, a conveyor extending transversely of said storage bins for feeding material into each of said storage bins, and means for transferring material from said first mentioned conveyor to said last mentioned conveyor.

45 50 7. Apparatus of the character described, comprising in combination, a plurality of digesters, a plurality of dump tanks positioned in line and arranged to receive material discharged from said digesters, draining means for each of said dump tanks, means for discharging drained material of low moisture content at a controlled rate from each of said dump tanks, and a common conveyor for receiving material as discharged 55 from each of said dump tanks and for transporting the material to a subsequent treating apparatus.

60 65 8. Apparatus of the character described, comprising in combination, a plurality of leaching tanks arranged in line, a conveyor

extending transversely of said tanks for receiving leached material discharged from each of said leaching tanks, a plurality of digesters arranged in line, a plurality of storage bins for said digesters positioned in line and in feeding relation with said digesters, a conveyor extending transversely of said storage bins for feeding material to each of said storage bins, means for transferring said material from said first mentioned conveyor to said second mentioned conveyor, a plurality of dump tanks arranged in line beneath said digesters for receiving material discharged therefrom, means for discharging material from each of said dump tanks, and a conveyor common to all said dump tanks for receiving material discharged therefrom and for conveying it to subsequent treating apparatus.

70 75 80 85 In testimony whereof I hereto affix my signature.

CHARLES S. HAMM.